

W. M. PAGE.

COMPOUND METAL AND PROCESS OF MAKING THE SAME.

APPLICATION FILED JUNE 23, 1911.

1,125,161.

Patented Jan. 19, 1915.



Inventor

Witnesses

H. C. Richter  
R. F. Steward

By

W. M. Page  
by  
K. P. McElroy  
Attorney

# UNITED STATES PATENT OFFICE.

WILLIAM MARSHALL PAGE, OF RIDLEY PARK, PENNSYLVANIA.

## COMPOUND METAL AND PROCESS OF MAKING THE SAME.

1,125,161.

Specification of Letters Patent.

Patented Jan. 19, 1915.

Application filed June 23, 1911. Serial No. 634,885.

*To all whom it may concern:*

Be it known that I, WILLIAM MARSHALL PAGE, a citizen of the United States, residing at Ridley Park, in the county of Delaware and State of Pennsylvania, have invented certain new and useful Improvements in Compound Metals and Processes of Making the Same, of which the following is a specification.

10 This invention relates to compound metals and processes of making the same; and it comprises a compound metal body having a copper body with a plurality of incorporated or embodied distributed isolated pre-  
15 formed copper-clad steel linear longitudinally arranged elements of relatively small diameter distributed therethrough and within its exterior surface, such copper-clad elements comprising layers or bodies of copper and steel united together by a weld union; and it comprises a process of making such conductors wherein a plurality of copper-clad rods, bars or the like elements having a weld-united copper sheath and steel core,  
20 and possessing the properties of drawn and worked metal, are placed in a mold in properly located, spaced and distributed arrangement and a body of copper or cupriferous alloy is cast around and among said rods in said mold to form a reinforced billet; the assemblage or billet being afterward worked down to the desired dimensions to secure a compound body of copper reinforced by embodied threadlike incorporated weld-  
25 coated steel threads weld-united thereto; the operation being repeated one or more times, if desired, by placing rods, bars, or the like of the metal so produced within a mold, casting in copper and working down anew;  
30 all as more fully hereinafter set forth and as claimed.

For many electrical purposes, as for hung and strung wires, it is desirable to provide a compound conductor comprising steel and copper, the steel giving the tensile strength and the copper conductivity. Until recently, however, it has been impossible to provide satisfactory material of this character. Unless the copper and steel be so  
35 welded together that they can be conjointly worked down and cannot part in use or seam apart, a steel cored compound wire of the two metals carrying, as has sometimes

been proposed, a relatively thick core of steel, is not durable or satisfactory in use. 55 Copper and steel have different rates of expansion, and if a wire carrying a copper sheath, for example, and a relatively large steel core be not welded together, under changes of temperature in use, the copper 60 tends to creep. The greater the proportionate thickness of the steel core as compared to the copper sheath the greater are these difficulties. Further, since copper and steel stand at widely different points in the 65 galvanic scale, the presence of a crevice or line of separation between two layers of these metals tends to accelerate corrosion, rapidly making the compound wire useless. With a heavy cored unwelded wire the 70 seam is a constant source of trouble. Aside from the opening of crevices or seams by the action of temperature changes, which will always occur with unwelded material, it is obvious that with relatively heavy and 75 stiff bodies of copper and steel, such as are produced in attempting to roll down together a heavy steel core in a heavy copper sleeve it is substantially impracticable to get the abutting surfaces into exact contact 80 at all points; and any point of separation or fault or flaw in a compound billet reappears in exaggerated dimensions in the wire made from it. And it is of course not practicable for wires intended for use out of doors to be composed of copper and naked steel wires stranded together, since in such an assemblage the steel rapidly rusts out. Recently however satisfactory compound 85 wire has been produced by welding together 90 copper and steel by methods such as are disclosed in Patent 853,716. A compound billet or ingot of copper and steel united by the process of that patent may be drawn to compound wire of any size desired and it 95 has been satisfactorily demonstrated that this wire is not subject to corrosion, galvanic action or parting. This material is ordinarily made with a central core of steel and a welded on sheath of copper, since for 100 exposed wires and the like there must be copper on the outside; the steel must not be exposed. For commercial purposes it is often made with a copper sheath having about 40 per cent. of the total sectional area, 105 the steel core representing the remaining 60

per cent. For many electrical purposes however it is desirable to have a higher conductivity than a 40 per cent. material can give and at times to have the steel located 5 elsewhere than centrally of the compound body though it must not be exposed; that is, must not occur on the exterior. Wire of such higher conductivity may be made from copper-steel billets formed according to the 10 process of the patent above referred to. But where conductivities as high as 60 to 70 per cent. are desired, it requires great skill to roll the billets properly to give a satisfactory product. For many wire purposes 15 where a wire is required to possess a given conductivity, a large diameter steel core gives greater strength and stiffness than is necessary, and at the same time adds surplus weight. Neither is a single central core of 20 steel the most advantageous form of reinforcement and particularly where it is desired to have a fairly flexible yet strong wire of high elastic limit. In order to secure a high tensile strength, a good grade of steel 25 is usually employed for the core and the wire making operations give it a temper, so that a steel cored wire is usually rather stiff and springy. For many electrical purposes it is desirable that the wire should be 30 mainly copper with reinforcing steel so distributed in it as to give a maximum tensile strength with a minimum weight of steel and a maximum conductivity and flexibility. For carrying heavy currents the greater the 35 percentage of copper that can be used in a wire of a given cross section the better, while at the same time the wire must be structurally strong. Any copper wire between poles is apt to sag and neck under the 40 influence of strains and temperature changes, since copper wire has a low elastic limit, and of course when stretched beyond this elastic limit, it does not recover its original section. If there be any necking at any point in the 45 wire the carrying power of the whole wire is reduced, while at the points of reduced section there is a proportional loss in tensile strength and there may be an undue development of heat. In all electrical wire and 50 material of this character it is desirable that the copper and steel shall be welded together, and while for the formation of a weld-union the presence of an alloyed area between the two metals seems to be necessary, yet the amount of iron occurring in 55 the main-body of the copper should be restricted to a minimum; there should be no penetration of iron beyond the necessary alloyed area into the main body of the copper. 60 The presence of a tenth of one per cent. of iron as an alloy in the main copper sheath reduces the conductive power of such copper for electrical current inordinately.

In the present invention I have devised an 65 improvement in compound conductors and

the processes of producing such conductors. I provide a wire having a number of discrete longitudinal steel threadlike bodies located near the periphery and spaced away from each other. This gives me a desirable type 70 of reinforcement, giving the wire a very high tensile strength for the amount of steel used. The absolute amount of steel in the wire required for a high tensile strength is much reduced with the reinforcing steel 75 thus distributed through the body of the copper as discrete threads of small diameter, and a much more flexible wire is obtained. In making the material, I use rods which have been previously coated with a weld- 80 united body of copper, and I cast copper around and among them to produce a compound reinforced billet. By using copper clad rods as reinforcing cores or bodies in producing such a reinforced billet, the cast 85 copper welds to the copper coating which itself is already welded to the steel, producing an integral body which can be drawn down in such a way as to reduce the included steel to threads of a very small diameter. There is no possibility of these threads separating from the body of the copper in the finished rod or wire. By using steel 90 bodies or rods carrying a preformed protective coating of pure copper, contamination of the cast copper by solution of iron in the operation of casting copper around the rods cannot of course occur. The solid metal with which the pure fluid copper comes into contact is itself pure copper. 100 And with the solid metal and the fluid metal both pure copper, it is easy to secure an integral union or weld therebetween. As the copper coating is already welded to the steel, 105 the billet is integral.

By first coating a steel billet with copper after the manner of Patent 853,716 and working it down to rods, rods may be produced carrying a welded-on substantial coating of pure copper, this coating being materially improved in physical character during the working operation. During the working an exceptionally strong metal is produced. The coating of the rods for this purpose may be advantageously about 40 110 per cent. of the total section. By locating as many such rods as are desired in a mold and casting copper among and around the spaced and isolated rods, a compound billet 115 ingot is produced carrying distributed, isolated preformed, copper-clad steel reinforcing elements. However the rods may be arranged or clustered, they should be spaced away from the mold to allow formation of a peripheral layer of copper containing no steel. The size of the rods and their number may be as desired, this depending on the amount of reinforcement required. On now 120 rolling and drawing down the compound billet to the size desired, the steel cores of 125

the rods are reduced to threads and a compound wire is produced having isolated strengthening threads of steel contained within and reinforcing it, these threads being within the periphery of the compound wire and so located as to give an outer protective layer of copper. For most purposes where a relatively flexible strong wire is desired in the finished material it is desirable 10 to have about 10 per cent. of steel; and this steel may occur as a few comparatively coarse threads or as a larger number of finer threads. The reinforcements may be located within the wire in any arrangement 15 desired; they may be clustered in any way or be a series of spaced, preformed, copper-clad steel threads located in annular arrangement in a layer near the periphery.

The coated rods or other shapes employed as core materials in the present invention are best of the character of material described in Patent 893,932, having a core of steel and a weld-united substantial coating of copper, the union being such as 20 to resist temperature changes and mechanical stresses and separation. Such material may as stated be made by the process of Patent 853,716, wherein steel is given a preliminary film coating by contacting with 25 supermolten or superheated copper and is thereafter united with a substantial body of cast copper. This cast copper should be pure. The material so produced should be worked down to the dimensions desired in 30 the present invention as by rolling to 3/8 inch rod or other shape where comparatively small compound billets, say round billets of about six to seven inches in diameter are to be made. The particular size 35 of the rods used of course depends both on the size of the billet to be produced and on the percentage of steel desired in the billet, and in the final wire, the number of threads of steel desired, etc. Their shape is also a 40 matter of choice. Whatever the shape of the rod this shape will be substantially preserved in the final wire; round rods giving round threads, oval rods giving oval threads, channeled rods giving channeled threads, 45 and so on. Where a maximum stiffness of the wire and minimum amount of steel is desired, it is sometimes best to use rods rolled in the shape of an I or T or a channel. But ordinarily, round, hexagonal, octago- 50 nal, etc., rods are best. It is in general desirable that the cores be about 1/2 inch to 3/8 inch in diameter where moderate sized billets are to be made. Where it is desired to obtain the steel directly as very fine 55 threads by a moderate reduction as in making coarse wire with fine reinforcements, instead of using 3/8 inch solid bars, a smaller size rod or bar may be substituted or copper clad wire may be stranded to produce 60 65 3/8 rope and lengths of this stranded ma-

terial employed. If an integral union of the preformed strengthening element with the cast copper is desired at the time of making the new compound wire, as is usually the case, the surface of such preformed clad metal reinforcing elements should be clean and metallic to enable it to unite easily therewith. The surface of the coated rods may be pickled with hydrochloric acid to form a little chlorid of copper thereon. This seems to aid in producing union between the cast copper and the coppered surface. If it be desired for any reason not to have a metallic union between the reinforcing elements and the cast copper, the surface of the former may be oxidized. Any convenient type of mold may be employed for the casting operation in making the compound billets or ingots. It is, however, often desirable to use a mold 25 of the type of that described in my copending application 607,338; a mold provided with means for maintaining an inert atmosphere of producer gas or nitrogen therein and having means for casting the copper 30 through restricted orifices near its top. A mold of this type prevents oxidation of the cores and of the metal cast in, and gives desirable material. 35

In making ordinary steel wire, the original bloom of 16 or 18 inches square is usually reduced to a 4-inch square billet but assuming, in order to make the manufacture of such wire comparable with that of the copper clad material used in this invention, 40 that the billet is a 6x6 billet, it would be reduced to a 3/8 rod in about 20 passes by hot rolling with not over 2 reheatings or heat treatments. It would then be cold drawn to No. 9 B. & S. wire in about 6 drafts. On 45 the other hand, in the manufacture of the material of the present invention, a 6x6 steel billet may be coated with copper to give an 8-inch square copper clad billet and then this reduced to 3/8 rod by operations involving about 22 passes by hot rolling and three reheatings or heat treatments. And 50 since the steel is rolled and worked inside a temperature-equalizing sheath of copper, it assumes a much more homogeneous, finer 55 grained and stronger structure than is possible to secure in rolling down naked steel. Partly for this reason and partly because of the heat treatments, copper clad rod and wire thus produced exhibit a very high tensile strength. Upon now cutting up 3/8 rods of this material, placing them in a mold of a shape and size to form, say, a 6 5/8 round billet, casting in copper to form 60 such a billet and reducing the billet to 3/8 rod, there may be 20 more hot rolling passes exerted on the included steel, with three reheatings or heat treatments. In drawing 65 this rod to No. 9 wire there may be 9 cold drafts. All this working down results in 70 75 80 85 90 95 100 105 110 115 120 125 130

an extraordinary improvement of the threadlike lines of steel included within the final compound wire. Such compound wire exhibits a tensile strength considerably in excess of what would be expected from the combined strengths of the cross sectional areas of copper and steel present. That is, the effect of incorporating steel threads in the copper body in the present manner is not merely additive as regards strength or, in other words, the tensile strength of a compound wire of the present invention is greater than the tensile strength of a steel wire having a cross sectional area equal to that of the steel in the compound wire, plus the tensile strength of a copper wire having a cross sectional area equal to that of the copper in the compound wire. The steel threads in this wire correspond in size to very fine, extraordinarily strong wires. Presuming the 3/8 compound thread reinforced rod produced as just described to be cold drawn to No. 9 wire, which will require about 9 drafts, the diameter of each steel thread in the wire will be about .00002 inches. Considering each steel thread as a wire, it may be stated that in the described process of converting the original steel into copper clad rod and then into steel threads in the new compound wire, each such thread wire will have received, say, 42 passes in hot rolling, 6 reheatings or heat treatments and 9 drafts with cold drawing. The steel in an all-steel wire of the same size as the compound wire (No. 9 B. & S.) would have received probably but two heat treatments, 20 passes by hot rolling and 6 or 7 drafts, cold drawing, and its tensile strength per unit of sectional area as compared to that of the steel of the threads of the compound wire, is markedly less. This mode of treatment may be carried as far as desired. After having made a compound primary billet of 3/8 copper coated rod with copper cast around and welded thereto, 3/8 rod rolled from this primary billet may be used as cores or reinforcements for a new secondary billet, made in the same way, which in turn may be reduced to 3/8 inch rod or wire; and so on. The number of these re-treatments may be almost indefinite. In each such treatment, of course, the steel is converted into finer and finer threads. Presuming 3/8 clad rods containing 60 per cent. steel to be used in making a 6 5/8 compound primary billet, this billet in turn reduced to 3/8 rod, and the new 3/8 rod in turn used as a core material for another or secondary billet, then this last billet on being drawn down to 3/8 rod would carry steel threads each of a diameter of approximately .00000066 inches and in a No. 9 wire therefrom, the diameter of each thread would be approximately .00000062 inches. Ordinarily, steel wire is seldom drawn below a

No. 40 size, but the several steel threads in the wire just described would be each about 1/50,000th of the size of No. 40 wire.

In making up what may be called, for the sake of clarity, a primary billet, of say 6 5/8 inches in diameter, to produce a primary wire having 10 per cent. steel, 54 copper clad 3/8 inch rods carrying about 60 per cent. steel may be used. If a secondary billet, that is a billet made by using rods rolled down from a primary billet such as just described, be required carrying 10 per cent. steel, then in making the primary billet about 130 of such 60 per cent. coated 3/8 rods may be used. These 130 rods will represent about 41 per cent. of the sectional area of the primary billet and with 60 per cent. steel in the rods the area of steel will be 25 per cent. In the secondary billet and in the wire drawn therefrom, using 130 rods in the primary billet and 130 primary rods in the secondary billet there will be 16,900 steel threads; or, strictly speaking, 16,900 copper clad steel threads. And the steel of these 16,900 threads together will represent about 10 per cent. of the area of the whole secondary wire. It may be taken as an accepted fact that with each new working there is a gradual increase in the strength and other desirable physical properties of steel, whether this working be hot or cold and especially in cold working as in wire drawing. Subsequent annealing never removes the effect of this working altogether. And in the present case, working is done under the most favorable conditions, because while the steel is being reduced to excessively fine threads (or the equivalents of wires,) yet these threads have been produced with a distribution and equalization of heat and pressure which is impossible to produce with naked steel in wire making. And this working is done under total exclusion of air. Furthermore, the effect of working and especially cold working on any metal is of course superficial; the hardening and strengthening only penetrate a given distance below the surface; with a comparatively large core of steel, most of the effect is in this outer layers. With fine threads of steel, in a billet or wire and with these threads a limited distance below the peripheral surface the steel receives the full effect of the working, and the more so since the copper in which the threads are embedded acts, in a way, as a fluid pressure transmitting body. The toughening effect of working is therefore transmitted to and affects the distributed steel threads in a more thorough way in each pass or draft than in an axially reinforced wire where the steel exists as a comparatively thick central core spaced away as far as possible from the working tool. With a given amount of steel existing as a plurality of distributed, iso-

lated relatively fine incorporated threads, a stronger and tougher wire can be made in a given number of passes, or, conversely, for a given strength and toughness, fewer 5 passes are necessary.

In the accompanying illustration I have shown more or less diagrammatically, means and materials within the described invention.

10 In this showing, Figure 1 is a vertical section of a mold containing clad metal rods and a body of cast copper; Fig. 2 is a transverse section of a reinforced primary billet; Fig. 3 is a similar section of a primary wire 15 such as may be drawn from the billet of Fig. 2; Fig. 4 shows a similar primary billet with reinforcing bodies in several annularly arranged sets; Fig. 5 is a similar view of a billet with the reinforcing bodies 20 clustered in the center; Fig. 6 is a similar view of a billet having the reinforcing rods in star-shaped alinement; Fig. 7 is a section of a secondary billet; and Fig. 8 is a vertical transverse section of a flat sheet 25 bar or billet adapted for making sheets and other flat articles.

In the showing of Fig. 1, element 1 is a mold set in base plate 2 and having a top 3 provided with pouring inlet 4. Gas inlet 30 5 allows the maintenance of an indifferent atmosphere in the mold during the pouring operation. Outlet 6 allows escape of gas. As shown, the mold contains a body of cast 35 copper 7 having embodied in it a plurality of rods of copper clad material, the steel core in these rods being marked 8, and the copper sheath 9.

In Figs. 2, 3, 4, 5 and 6 the copper body is marked 7 and the reinforcing rods 10.

40 In Fig. 7 the copper body (7) contains embodied primary rods 11, each of such primary rods containing a plurality of steel threads 12.

For conductor wire, and particularly wire 45 from a primary billet, it is better to use copper clad rods of the character described carrying a substantial coat of copper, rather than rods which have been merely alloyed by dipping, as there is less risk of 50 contamination of the cast in copper by iron.

As stated, the reinforcing bodies or rods used may be square, flat, round, oval, hexagonal, octagonal, channeled, etc. If stranded 55 copper clad wire in rope or cable form be employed, as by using sections of such a cable in lieu of rods, the fineness of the steel threads in a primary billet or wire can be made as great as desired. But a stranded cable of clad wire is more expensive than a 60 rolled rod. Where reinforced brass, bronze, or the like cupriferous metal is desired, brass, bronze or the like may be cast around the clad metal reinforcing rods in the manner described for the casting of copper. 65 The billet may afterward be worked down

in the same manner as the reinforced copper. The extreme fineness of the steel threads insures that even if one thread should not be welded to the copper, there will be no substantial avenue for the penetration of moisture, etc. And with the multiplicity of spaced and isolated threads any break or other injury to one does no particular harm since the others will not be affected.

Since the material of the present invention is to be a reinforced copper, that is copper reinforced with distributed threads of steel, rather than a copper clad steel, the amount of copper for most purposes should always be relatively great as compared with 70 the amount of steel, at least in the finished article. For the present purposes, 10 to 15 per cent. steel in the finished article is usually amply sufficient to give a very high tensile strength while affording material 75 which is still, as regards all other properties, substantially copper. With greater amounts of steel, the properties begin to vary more from those of copper; and while this high steel material is desirable for some purposes, 80 for which it displays unique combinations of properties, yet for high conductivity, high strength, flexible conductors, the 10 per cent. material is desirable. The more steel threads 85 the total 10 per cent. represents the more 90 flexible is the wire. Material consisting of a copper body carrying higher percentages, up to 30 or 40 per cent., of fine steel threads is useful for some purposes. A 30 per cent. material carrying the incorporated steel in 95 the form of several hundred or thousand isolated distributed threads has very great tensile strength and relative flexibility as compared with stranded ropes, cables and the like. The steel threads are usually much 100 finer and stronger than steel wire can be 105 commercially produced and are spaced and united by the layers of copper in a way which gives the assemblage special properties.

110 In place of copper clad steel rods or threads as reinforcing members, bronze clad, brass clad, or aluminum clad steel may be employed to produce primary, secondary, tertiary billets, and so on, in the way described for copper clad steel rods. Ordinarily however, copper clad steel is most convenient to use and gives the most satisfactory results.

115 While my invention is particularly useful 120 in making rods, wires, and the like, and particularly for conductor purposes, it is also applicable for the manufacture of sheets, tubes and other shapes. For many purposes for which copper is used in the arts, because of its non-corrodibility, such as evaporating devices and the like, it is desirable to have it of a somewhat stronger character. The size of a vacuum pan, for example, is 125 limited by the structural strength of copper 130

in available sizes. A vacuum pan must withstand atmospheric pressure and if the pan be over a given size, copper sheets cannot be relied upon to furnish the strength unless 5 of undue thickness and weight. Metal sheets for such purposes however must be like copper, capable of being worked into shape under the hammer; the metal must be malleable and flow under the tool. By reinforcing copper with steel in the present invention sheets can be obtained which combine 10 a high tensile strength with a flowability like that of copper. For this purpose instead of using only longitudinal reinforcing 15 elements it is better to have reinforcing elements in two directions. That is, instead of merely clustering longitudinal rods in a mold and casting copper about them, it is better to use rods arranged in two directions. 20 The rods may, and very useful for many purposes, be interlaced in a sort of open fabric. Presuming that strengthening rods of material such as described, be woven into a sort of loose or open fabric, that is in 25 right-angled arrangement, copper cast about them to form a compound billet and then rolled down into sheets, an article will be secured which is substantially copper so far as its hammering properties are concerned, but 30 nevertheless has a greater degree of strength than copper alone can have. If the reinforcements be, as is preferable, each of relatively small diameter as regards the body of copper, on cutting the new reinforced sheet 35 to sizes such as are desired, there will be merely spots of steel exposed; and these spots may, and usually will be too small in diameter to allow corrosion to penetrate far by capillary penetration. They may, of 40 course, be touched with a soldering iron. The reinforced sheet may also be punched and drilled to receive rivets and the like without any substantial exposure of the reinforcing metal.

45 Reinforced bars or sheets such as described, which may have reinforcements distributed through the bar or sheet in one or more planes, may of course be converted into structural elements, such as T's, I's, chan-

50 nels, cross-sectioned elements, etc. For such material of course perforated plates of strong metal, "expanded metal," or electrically welded woven screen as well as ordinary woven screen material may be em-

55 ployed. But the product, using such materials, does not have the reinforcements spaced and isolated from each other at all points. In Fig. 8 I have shown in cross section a flat billet adapted for sheets and

60 other flat shapes and consisting of a copper body 7 having embodied in it a plurality of rods 8 and 8<sup>a</sup> arranged in two directions and at right angles with each other.

What I claim is:—

65 1. A reinforced copper article comprising

a body of copper and a plurality of isolated linear elements of a stronger metal incorporated with and distributed through said body of copper, said linear elements being spaced away from and in substantially parallel alinement with an outer wall of such copper body. 70

2. A reinforced copper article comprising a body of copper and a plurality of isolated linear elements of steel incorporated with 75 and distributed through said body of copper, said elements of steel being spaced away from and in substantially parallel alinement with an outer wall of such copper body. 80

3. A reinforced copper article comprising a body of copper and a plurality of isolated linear elements of steel incorporated with and distributed through said body of copper, and spaced away from and in substantially parallel alinement with an outer wall of said copper body, said linear elements carrying a preformed weld-united coating 85 of copper and having the characteristics of worked metal. 90

4. A reinforced copper article comprising a body of copper and a plurality of isolated linear elements of steel incorporated with and distributed through said body of copper and spaced away from and in substantially parallel alinement with an outer wall of said copper body, said linear elements carrying a preformed weld-united coating 95 of copper and having the characteristics of worked metal, and the steel being integrally 100 united to said body of copper through said coating of copper. 105

5. A reinforced copper article comprising a body of copper and a plurality of isolated threadlike linear elements of a stronger metal incorporated with and distributed through said body of copper, each threadlike element being of a diameter relatively minute as compared with the sectional area 110 of such copper body, and being spaced away from and in substantially parallel alinement with an outer wall of such copper body. 115

6. A reinforced copper article comprising a body of copper and a plurality of isolated threadlike linear elements of steel incorporated with and distributed through said body of copper, each steel element being of a diameter relatively minute as compared with the sectional area of such copper body, and being spaced away from and in substantially parallel alinement with an outer wall of such copper body. 120

7. A reinforced copper article comprising a body of copper and a plurality of isolated threadlike linear elements of steel incorporated with and distributed through said body of copper, each steel element being of a diameter relatively minute as compared with the sectional area of such copper body, spaced away from and in substantially par- 125

130

- 5      14. The process of making reinforced copper articles which comprises placing a plurality of steel bodies having a welded-on coating of copper in spaced and isolated arrangement within a mold and at a distance from its walls, casting copper into said mold and extending the billet so formed. 70
- 10     15. The process of making reinforced copper articles which comprises placing a plurality of bodies comprising weld-united copper and steel in spaced and isolated arrangement within a mold and at a distance from its walls, casting copper into said mold and extending the billet so formed to produce 75 rods. 80
- 15     16. The process of making reinforced copper articles which comprises placing a plurality of bodies comprising weld-united copper and steel in spaced and isolated arrangement within a mold and at a distance from its walls, casting copper into said mold, extending the billet so formed to produce rods, placing said rods in a mold in spaced arrangement and casting copper 85 thereabout to produce a secondary billet. 90
- 20     17. The process of making reinforced copper articles which comprises placing a plurality of bodies comprising weld-united copper and steel in spaced and isolated arrangement within a mold and at a distance from its walls, casting copper into said mold, extending the billet so formed to produce rods, placing a plurality of said rods in a mold in spaced arrangement and casting copper 95 thereabout to produce a secondary billet and extending said secondary billet. 100
- 25     18. The process of making reinforced copper articles which comprises casting molten copper against and around a plurality of spaced steel bodies coated with welded-on copper, and allowing said molten copper to set thereagainst. 105
- 30     19. The process of making reinforced copper articles which comprises placing a plurality of bodies comprising steel in spaced and isolated arrangement within a mold and at a substantial distance from its walls, and casting copper into said mold. 110
- 35     20. The process of making reinforced copper articles which comprises casting molten copper among and around a group of spaced bodies comprising steel, and allowing said molten copper to solidify into a body uniting 115 said spaced bodies and forming a substantial layer surrounding said group as a whole. 120
- 40     21. The process of making reinforced copper articles which comprises casting molten copper among and around a group of spaced bodies comprising steel, and allowing said molten copper to solidify into a body uniting 125 said spaced bodies and forming a substantial layer surrounding said group as a whole, the ratio of copper to steel in the 130
- 45     13. The process of making reinforced copper articles which comprises placing a plurality of bodies of weld-united copper and steel in spaced and isolated arrangement within a mold and at a distance from its walls and casting copper into said mold. 135
- 50     12. A reinforced copper article comprising a body of copper and a plurality of distributed and isolated linear reinforcing elements of metal spaced away from and in substantially parallel alinement with an outer wall of said body of copper, each such reinforcing body comprising a plurality of parallel threads of weld-united copper and steel. 140
- 55     11. A reinforced copper article comprising a body of copper and a plurality of distributed and isolated linear reinforcing elements of metal spaced away and in substantially parallel alinement with an outer wall of said body of copper, each such reinforcing body comprising a plurality of parallel threads of weld-united copper and steel. 145
- 60     10. A reinforced copper article comprising a body of copper and a plurality of distributed and isolated linear reinforcing elements of metal incorporated with said body of copper, and in substantially parallel alinement with an outer wall thereof, each such reinforcing element comprising a plurality of threads of steel in parallel alinement. 150
- 65     9. A reinforced copper article comprising a body of copper and a plurality of distributed and isolated linear reinforcing elements of metal spaced away from and in substantially parallel alinement with an outer wall of said copper body, each such reinforcing element comprising a plurality of threads of stronger metal in parallel alinement. 155

- resulting reinforced article being relatively large.
22. The process of making reinforced copper articles which comprises placing a plurality of bodies comprising steel having a coating of a softer metal united thereto in spaced and isolated arrangement within a mold and at a substantial distance from its walls, and casting copper into said mold.
- 10 23. A reinforced copper article comprising a body of copper and a plurality of

isolated linear elements of steel incorporated therewith and distributed therethrough, the copper being present in predominating quantity.

In testimony whereof, I affix my signature in the presence of two subscribing witnesses.

15

WILLIAM MARSHALL PAGE.

Witnesses:

K. P. McELROY,  
FRANK R. CHAMBERS, Jr.